

Dec. 30, 1969

T. NILSSON ET AL

3,486,969

PROCESS FOR THE TREATING OF WOOD CHIPS WITH FUNGI TO ENHANCE  
ENZYMATIIC HYDROLYSIS OF THE RESINOUS COMPONENTS

Filed July 19, 1966



1

3,486,969

**PROCESS FOR THE TREATING OF WOOD CHIPS  
WITH FUNGI TO ENHANCE ENZYMATIC HYDROLYSIS OF THE RESINOUS COMPONENTS**

Thomas Nilsson, Stockholm, and Anders Assarsson,  
Ornskoldsvik, Sweden, assignors to Mo och  
Domsjö Aktiebolag, Ornskoldsvik, Sweden, a corporation of Sweden

Filed July 19, 1966, Ser. No. 566,309

Claims priority, application Sweden, July 20, 1965,  
9,591/65

Int. Cl. D21b 1/02

U.S. CL. 162—72

4 Claims

**ABSTRACT OF THE DISCLOSURE**

A dispersion of selected fungi is added to wood chips which are stored prior to further processing such as by chemical digestion to form pulp. The chips are subjected to enzymatic hydrolysis induced by the fungi while minimizing microbial action on cellulose and hemicellulose in the wood.

The present invention relates to a process for storing wood chips whereby said chips are stacked in piles, and to an arrangement for carrying out the method.

When preparing cellulose pulp the resin components present in the wood give rise to certain problems being difficult and costly to remove, causing disturbances in production and impairing the quality of the finished product. Resin from, predominantly, hardwood and softwood comprises hydrocarbons, waxes (esters between fatty acids and higher alcohols), glycerides and higher alcohols. Furthermore, present in softwood are diterpene acids (resin acids) and diterpene aldehydes. One method of facilitating the removal of these compounds is to store the barked or unbarked wood as round logs, on land or in water. When storing in water an enzymatical hydrolysis of the glycerides of the resin takes place. When storing on dry ground an autoxidation of saturated resin components takes place, in addition to the hydrolysis of glycerides, when the wood dries out. Both enzymatical hydrolysis and autoxidation facilitate removal of the resin in later pulp manufacturing processes. Round-timber storage, however, takes a long time and, furthermore, gives rise to a certain decomposition of cellulose and hemicellulose in the wood. To reduce these disadvantages investigations have been made as to the possibility of storing wood in the form of piles of chips, in which an enzymatical hydrolysis, autoxidation and a biological decomposition of all resin components takes place. However, when adopting these means a biological breakdown of cellulose and hemicellulose also takes place, which causes the loss of valuable wood substances. Decomposition of resin has been discovered to give rise to resin losses which can substantially be attributed to the fatty acids released on the enzymatical hydrolysis of fats and waxes, which have thus been subjected to biological decomposition reactions. The enzymatical hydrolysis of the waxes is an advantage which is not obtained in any other method of storing wood. The waxes are extraordinarily difficult to remove during the pulping process due to the fact that their ester linkages are sterically hindered which make saponification almost impossible. This is illustrated by the fact that waxes in wood which is digested according to the sulphate method to 90%

2

survive this treatment without being saponified and that the alkali treatment to which the pulp is subjected in the bleaching plant influences the ester linkages of the waxes to a still less degree. The waxes therefore enter into the finished pulp product and impair its quality. The present invention is built on the hypothesis that microorganisms present in stacks of wood chips have a decisive significance for the aging of the resins and the decomposition of cellulose and hemicellulose. The method according to the invention is characterized in that during the process of stacking the piles of wood chips, said chips are supplied with a culture of one or more microorganisms which break down the resin components present in the chips but do not decompose the cellulose, said microorganisms, moreover, preferably having an inhibiting effect on other cellulose and hemicellulose decomposing microorganisms normally appearing in the pile of wood chips.

By these means it is possible to obtain an appreciably shortened storage time in comparison with the storage of wood as logs whilst at the same time obtaining an extraordinarily good resin ageing without the simultaneous decomposition of cellulose or hemicellulose, and to remove the waxes so disadvantageous to the pulp processes. The microorganisms may also possibly be added together with a nutritional salt solution. The inhibition of cellulose or hemicellulose decomposing microorganisms may in principle be effected in three different ways. Firstly it is possible to elect to add such a microorganism which, at the same time as it decomposes the resin constituents, inhibits the cellulose and hemicellulose decomposing microorganisms by generating such a high temperature in the pile of wood chips that the latter microorganisms are prevented from propagating. In this respect the said microorganisms can only withstand a temperature of, at the most approximately 50° C. Another method is to add a resin decomposing micro-organism which by an anti-biotic effect prevents the cellulose and hemicellulose decomposing micro-organisms from propagating. A third method is, at the same time as the specific resin decomposing micro-organism is added, to add a substance which has an inhibiting effect on the cellulose and hemicellulose decomposing micro-organisms, e.g. nickel sulphate. Naturally it is also possible to use combinations of these three methods of inhibiting cellulose and hemi-cellulose decomposing micro-organisms.

Suitable micro-organisms which can be used according to the present invention are fungi, which completely or partly lack the ability of producing active celluloses on wood but which can produce esterases such as lipases, sterolases, sterolesterases, fatty alcoholases, fatty alcohol esterases, terpene alcoholases, and terpene alcohol esterases, i.e. the enzymes which break down the ester linkages in the wood resin. It is, moreover, advantageous if they produce enzyme systems which break down the carbon chains of the resin compounds by oxidation. The micro-organisms should preferably also be sporulating since the spores can then easily be added to the wood chips in the form of an aqueous dispersion, but if the micro-organisms are constituted of non-sporulating fungi it is naturally also possible to break down the same prior to adding said organisms. The said micro-organisms should suitably also be resistant to low temperatures, to enable them to be used when storing wood chips in winter.

Examples of suitable resin decomposing micro-organisms which do not produce active cellulases on wood to

any appreciable degree, and which inhibit cellulose and hemicellulose decomposing micro-organisms by developing such a high temperature in the pile of wood chips that said micro-organisms cannot propagate are, i.a.:

- (1) *Humicola grisea* var. *thermoidea*, characterized by Cooney-Emerson
- (2) *Humicola stellata*, ch. by Bunce
- (3) *Humicola insolens*, ch. by Cooney-Emerson
- (4) *Humicola languinosa*, ch. by Griffon-Maublanc-Bunce
- (5) *Talaromyces duponti*, ch. by Griffon-Maublanc-Cooney-Emerson
- (6) *Thermoascus aurantiacus*, ch. by Miehe
- (7) *Mucor pusillus*, ch. by Lindt
- (8) *Mucor miehi*, ch. by Cooney-Emerson
- (9) *Malbranchea pulchella*, Saccardo-Penzig var. *sulfurea*, ch. by Miehe
- (10) *Myriococcum albomyces*, ch. by Cooney-Emerson
- (11) *Sporothrichum thermophile*, ch. by Apinis
- (12) *Allescheria terrestris*, ch. by Apinis
- (13) *Torula thermophila*, ch. by Cooney-Emerson
- (14) *Chaetomium thermophile*, ch. by La Touche
- (15) *Stilbella thermophile*, ch. by Fergus
- (16) *Aspergillus fumigatus*, ch. by Fresenius

Examples of suitable resin decomposing micro-organisms which do not produce active cellulases on wood and which inhibit cellulose and hemicellulose decomposing micro-organisms by antibiosis effect are i.a. the following:

- (17) *Trichoderma lignorum*, ch. by Tode-Harz
- (18) *Gliocladium roseum*, ch. by Link-Thom
- (19) *Gliocladium deliquescens*, ch. by Sopp
- (20) *Penicillium funiculosum*, ch. by Thom
- (21) *Penicillium roqueforti*, ch. by Thom
- (22) *Penicillium rubrum*, ch. by Stoll
- (23) *Gliocladium viride*

Other suitable fungi for use according to the invention, associated with any of said groups are the following:

- (24) Penicillium, our designation B76-1, a new species being characterized
- (25) *Dactyliomyces thermophilus*
- (26) *Rhizopus arrhizus*
- (27) *Byssochlamys*, our designation M 243 II, a new species being characterized
- (28) Penicillium, our designation P 116-I, a new species being characterized

A suitable apparatus for applying the method is shown diagrammatically in the figure. A plant for building a pile of wood chips is shown in the form of a blower machine 1, a pneumatic conveying duct 2, a chip hopper 3 with a discharge device (cell feeder) 4 connected to the duct 2. A tank 5 intended to contain a slurry of micro-organisms is connected via conduits 8 with a pump 6 and an overflow valve 7 in connection with nozzles 9 in the duct 2 on both sides of the junction where the cell feeder 4 is

connected to the duct 2. The slurry is injected into the chips by means of nozzles 9, while they are being transported to the storage site along the duct 2. The following examples illustrate the invention:

#### Example 1

Wax from spruce wood was isolated by extraction of spruce chips with ethanol-benzene (1:2), evaporation, extraction with ethyl ether and agitation of the ether-soluble portion with KOH, whereby the acid substances present in the resin were converted into their water-soluble potassium salts, which were separated. The neutral portion was subjected to chromatography on a silicagel column and the eluate containing wood waxes was mixed, subsequent to evaporation, with a nutritional salt solution containing the following ingredients:

|                                           | Mg. |
|-------------------------------------------|-----|
| $\text{KH}_2\text{PO}_4$                  | 350 |
| $\text{KHPO}_4$                           | 150 |
| $\text{NH}_4\text{NO}_3$                  | 500 |
| $\text{MgSO}_4 \cdot 7\text{H}_2\text{O}$ | 100 |
| Fe citrate                                | 20  |
| Yeast extract                             | 10  |
| Distilled water, 1000 ml.                 |     |

The concentration of resin in the nutritional salt solution constituted 1 mg./ml., and 30 ml. of the obtained emulsion was used for each test. 1 mg. of pure cultures of various micro-organisms according to the invention were injected into or on the emulsions, under the conditions which can be seen from Table 1, after which decomposition of the wax was determined. These micro-organisms were isolated from wood samples taken from wood chip piles by sterile transfer to agar plate cultures, wherefrom the separate micro-organisms were separated from the various colonies obtained and re-cultivated on agar plates. The spores from the thus re-cultivated micro-organisms were isolated by flushing with water.

TABLE 1

| Micro-organism                                | Temp.<br>° C. | Days | Agitated<br>culture | Stationary<br>culture | Wax decomposi-<br>tion             |
|-----------------------------------------------|---------------|------|---------------------|-----------------------|------------------------------------|
| <i>Penicillium</i><br><i>roqueforti</i> .     | 25            | 4    | +                   | -----                 | No trace of wax.                   |
| <i>Penicillium</i><br><i>funiculosum</i> .    | 25            | 8    | +                   | -----                 | Certain wax de-<br>composition.    |
| <i>Byssochlamys</i><br>M 243-II.              | 45            | 16   |                     | +                     | No trace of wax.                   |
| <i>Trichoderma</i><br><i>lignorum</i> .       | 25            | 8    | +                   | -----                 | Certain wax de-<br>composition.    |
| <i>Rhizopus</i><br><i>arrhizus</i> .          | 50            | 4    | +                   | -----                 | Wax consumption<br>and growth.     |
| <i>Dactyliomyces</i><br><i>thermophilus</i> . | 50            | 4    | +                   | -----                 | Do.                                |
| <i>Penicillium</i> B-76-I                     | 50            | 4    | +                   | -----                 | Wax decomposi-<br>tion and growth. |
| <i>Sporothrichum</i><br><i>thermophile</i> .  | 50            | 4    | +                   | -----                 | Do.                                |
| <i>Allescheria</i><br><i>terrestris</i> .     | 50            | 4    | +                   | -----                 | Do.                                |

The test shows that the above micro-organisms, which were all isolated from piles of wood chips, are capable of developing, using wax present in the nutritional solution as a source of carbon. The decomposition of wax which occurs when storing wood chips can thus be attributed to certain of the micro-organisms which are developed in the pile of chips.

#### Example 2

The ability, exhibited by some of the micro-organisms according to the invention, of selectively decomposing wood resin, primarily the waxes, and at the same time inhibiting the growth of other micro-organisms was determined by spraying wood chips with an aqueous dispersion of micro-organisms and analysis of the wood after a certain cultivating time. The wood chips were supplied with approximately  $10^{10}$  spores per kg. wood by spraying. The samples were stored for 0-60 days at two different temperatures, 35° C. or 50° C., depending on whether the organism was a high-temperature organism or low-

temperature organism. The samples were then extracted with ethyl alcohol and benzene in the ratio of 1:2, after which the extract was evaporated and treated with ethyl ether. The ether-soluble portion was made up of the resin remaining in the wood. This was agitated with KOH, acid substances (free fatty acids and resin acids) present in the resin being converted into water-soluble potassium salts, which were separated. The remaining ether solution was examined quantitatively and qualitatively chromatographically on its content of hydrocarbons, waxes, triglycerides, higher alcohols and other substances. At the same time completely untreated chips were analysed, said chips having been stored under corresponding conditions (control). The result can be seen from Table 2.

were placed at a level of 5 meters above the ground. At the same time 5 sacks containing untreated wood chips removed direct from the storage container were placed at the same level, for checking purposes.

The weight of the chips and the bulk density, extract content DKM, lignin content, pentosan content, carbohydrate composition and solids content of the chips in each sack were determined beforehand. Two months later the pile was broken down and the sacks removed, after which the above analyses were repeated. Temperature development in the sacks during storage was determined at various levels. Each chip portion placed in the pile was test cooked according to the sulphate method under standard conditions to 35 cp. viscosity, after which the

TABLE 2

| Definition                                                   | Control            |       |                           |       |                           |       |                             |       | <i>Rhizopus arrhizus</i>      |       |                              | Byssochlamys M 243-II |       |  |
|--------------------------------------------------------------|--------------------|-------|---------------------------|-------|---------------------------|-------|-----------------------------|-------|-------------------------------|-------|------------------------------|-----------------------|-------|--|
|                                                              | 0                  | 17    | 17                        | 30    | 30                        | 60    | 60                          | 30    | 50                            | 60    | 17                           | 30                    | 60    |  |
| Storage time, days.....                                      |                    |       |                           |       |                           |       |                             |       |                               |       |                              |                       |       |  |
| Storage temp., °C.....                                       | 35                 | 35    | 50                        | 35    | 50                        | 30    | 50                          | 30    | 50                            | 60    | 50                           | 50                    | 50    |  |
| EtOH/Benzene (1:2) extract.....                              | 3.248              | 2.645 | 2.676                     | 2.616 | 1.735                     | 3.395 | 2.087                       | 1.721 | 1.679                         | 2.499 | 2.114                        | 1.507                 | 1.507 |  |
| Insoluble in ether, percent of wood.....                     | 1.72               | 1.068 | 1.139                     | 1.728 | 1.050                     | 2.422 | 1.232                       | 1.089 | 1.064                         | 1.304 | 1.291                        | 0.927                 | 0.927 |  |
| Soluble in ether, percent of wood.....                       | 1.53               | 1.139 | 1.006                     | 0.888 | 0.685                     | 0.974 | 0.856                       | 0.633 | 0.616                         | 0.829 | 0.823                        | 0.580                 | 0.580 |  |
| Neutral substances, percent of wood.....                     | 1.024              | 0.541 | 0.474                     | 0.405 | 0.355                     | 0.380 | 0.311                       | 0.344 | 0.295                         | 0.472 | 0.424                        | 0.311                 | 0.311 |  |
| Hydrocarbons, percent of wood.....                           | 0.046              | 0.018 | 0.023                     | 0.018 | 0.015                     | 0.015 | 0.013                       | 0.011 | 0.012                         | 0.025 | 0.018                        | 0.011                 | 0.011 |  |
| Waxes, percent of wood.....                                  | 0.177              | 0.115 | 0.110                     | 0.083 | 0.073                     | 0.059 | 0.029                       | 0.045 | 0.026                         | 0.131 | 0.078                        | 0.037                 | 0.037 |  |
| Triglycerides, percent of wood.....                          | 0.532              | 0.106 | 0.061                     | 0.068 | 0.020                     | 0.092 | 0.062                       | 0.062 | 0.069                         | 0.075 | 0.075                        | 0.075                 | 0.075 |  |
| Higher, alcohols, percent of wood.....                       | 0.116              | 0.139 | 0.146                     | 0.151 | 0.135                     | 0.109 | 0.171                       | 0.134 | 0.171                         | 0.126 | 0.143                        | 0.167                 | 0.167 |  |
| Remainder, percent of wood.....                              | 0.150              | 0.164 | 0.185                     | 0.085 | 0.114                     | 0.103 | 0.096                       | 0.091 | 0.087                         | 0.131 | 0.112                        | 0.097                 | 0.097 |  |
| Free acids, percent of wood.....                             | 0.514              | 0.598 | 0.532                     | 0.483 | 0.380                     | 0.594 | 0.545                       | 0.289 | 0.321                         | 0.357 | 0.399                        | 0.259                 | 0.259 |  |
| Free fatty acids, percent of wood.....                       | 0.086              | 0.086 | 0.086                     | 0.086 | 0.086                     | 0.086 | 0.086                       | 0.086 | 0.086                         | 0.086 | 0.086                        | 0.091                 | 0.091 |  |
| Resin acids, percent of wood.....                            | 0.320              | 0.320 | 0.320                     | 0.320 | 0.320                     | 0.320 | 0.320                       | 0.320 | 0.320                         | 0.320 | 0.320                        | 0.137                 | 0.137 |  |
| Loss in weight percent of original wood, probable value..... | 0.95               | 2.29  | 1.23                      | 4.77  | 4.9                       | 4.7   | 4.58                        | 2.6   | 1.23                          | 1.95  | 3.8                          | 3.8                   | 3.8   |  |
| Lignin acc. to Klason.....                                   | 28.0               | 27.8  | 28.1                      | 27.07 | 27.33                     | 28.33 | 28.12                       | 27.43 | 28.69                         | 28.5  | 27.28                        | 29.49                 | 29.49 |  |
| Definition                                                   | Penicillium P116-I |       | <i>Gliocladium viride</i> |       | <i>Penicillium rubrum</i> |       | <i>Trichoderma lignorum</i> |       | <i>Penicillium roqueforti</i> |       | <i>Aspergillus fumigatus</i> |                       |       |  |
| Storage time, days.....                                      | 30                 | 60    | 30                        | 60    | 30                        | 60    | 30                          | 60    | 17                            | 30    | 60                           | 30                    | 60    |  |
| Storage temp., °C.....                                       | 35                 | 35    | 35                        | 35    | 35                        | 35    | 35                          | 35    | 35                            | 35    | 35                           | 50                    | 50    |  |
| EtOH/Benzene (1:2) extract.....                              | 2.751              | 1.865 | 2.070                     | 1.900 | 1.972                     | 2.208 | 2.345                       | 1.907 | 3.112                         | 2.084 | 2.012                        | 2.316                 | 1.734 |  |
| Insoluble in ether, percent of wood.....                     | 1.890              | 0.921 | 1.139                     | 1.095 | 1.117                     | 1.457 | 1.258                       | 1.091 | 1.998                         | 1.188 | 1.082                        | 1.435                 | 1.094 |  |
| Soluble in ether, percent of wood.....                       | 0.861              | 0.944 | 0.932                     | 0.806 | 0.855                     | 0.751 | 1.087                       | 0.816 | 1.114                         | 0.896 | 0.930                        | 0.881                 | 0.639 |  |
| Neutral substances, percent of wood.....                     | 0.399              | 0.487 | 0.437                     | 0.391 | 0.448                     | 0.397 | 0.493                       | 0.375 | 0.509                         | 0.464 | 0.390                        | 0.489                 | 0.235 |  |
| Hydrocarbons, percent of wood.....                           | 0.011              | 0.017 | 0.012                     | 0.013 | 0.016                     | 0.017 | 0.047                       | 0.010 | 0.018                         | 0.011 | 0.013                        | 0.019                 | 0.017 |  |
| Waxes, percent of wood.....                                  | 0.074              | 0.090 | 0.056                     | 0.059 | 0.084                     | 0.065 | 0.087                       | 0.058 | 0.131                         | 0.071 | 0.063                        | 0.102                 | 0.022 |  |
| Triglycerides, percent of wood.....                          | 0.085              | 0.083 | 0.089                     | 0.071 | 0.083                     | 0.080 | 0.087                       | 0.078 | 0.107                         | 0.085 | 0.083                        | 0.069                 | 0.069 |  |
| Higher alcohols, percent of wood.....                        | 0.110              | 0.162 | 0.109                     | 0.145 | 0.130                     | 0.127 | 0.166                       | 0.119 | 0.147                         | 0.141 | 0.144                        | 0.155                 | 0.131 |  |
| Remainder, percent of wood.....                              | 0.119              | 0.136 | 0.172                     | 0.102 | 0.136                     | 0.108 | 0.107                       | 0.109 | 0.107                         | 0.156 | 0.088                        | 0.144                 | 0.065 |  |
| Free acids, percent of wood.....                             | 0.462              | 0.468 | 0.495                     | 0.415 | 0.407                     | 0.354 | 0.594                       | 0.442 | 0.605                         | 0.432 | 0.540                        | 0.392                 | 0.404 |  |
| Free fatty acids, percent of wood.....                       | 0.125              | 0.125 | 0.125                     | 0.125 | 0.112                     | 0.164 | 0.193                       | 0.271 | 0.129                         | 0.129 | 0.129                        | 0.213                 | 0.213 |  |
| Resin acids, percent of wood.....                            | 0.254              | 0.254 | 0.254                     | 0.254 | 0.193                     | 0.271 | 0.193                       | 0.271 | 0.129                         | 0.129 | 0.129                        | 0.159                 | 0.159 |  |
| Loss in weight percent of original wood, probable value..... | 5.25               | 7.4   | 3.07                      | 1.5   | 2.46                      | 2.6   | 0.67                        | 2.7   | 1.51                          | 0.45  | 2.9                          | 0.89                  | 0.9   |  |
| Lignin acc. to Klason.....                                   | 27.33              | 28.66 | 27.47                     | 29.45 | 28.43                     | 28.91 | 28.57                       | 28.75 | 27.9                          | 27.79 | 29.13                        | 28.17                 | 28.87 |  |

As can be seen from the tables the decomposition of resin is considerably improved when applying the invention, in comparison with conventional methods of storing wood chips (compare "soluble in ether" in Table 2, line 3). For example the micro-organism Byssochlamys M 243-II gives an approximately 20% improvement in this respect. The amount of residual wax with the organisms used in the example was substantially unchanged whilst the loss of wood was greatly reduced.

### Example 3

A pile of chips 25 x 25 x 10 meters in dimension (2000 m.<sup>3</sup>) was built by means of the apparatus shown in the figure, said apparatus comprising a blower machine 1, a pneumatic conveying duct 2, a supply container for wood chips 3, in the lower portion of which was arranged a discharge device sealing against the supply container (cell feeder) 4. From a tank 5 with a capacity of 200 litres and containing 15.10<sup>11</sup> slurred spores of the micro-organisms *Rhizopus arrhizus* (high-temperature fungus) and *Gliocladium viride* (low-temperature fungus), the slurry was pumped by pump 6 via the over-flow valve 7 through the line 8 to the nozzles 9 arranged on both sides of the cell feeder into the pneumatic transport duct 2 at the same time as wood chips were fed into the said pneumatic transport duct. The slurry was delivered in an amount of 53 litres per hour whilst the chips were fed in at a speed of approximately 50 m.<sup>3</sup>/hour. To determine the loss of wood, five sample sacks of wood chips

obtained pulp was bleached according to the following schedule.

| 50 | Chlorine | Charging, percent | Time in mins. | Temp., °C. | Pulp consistency | pH   |
|----|----------|-------------------|---------------|------------|------------------|------|
|    | 1.030    |                   | 30            | 20         | 3                |      |
|    | 4        |                   | 120           | 85         | 6                |      |
| 55 | 1.2      |                   | 120           | 80         | 6                | 4.5  |
|    | 1.5      |                   | 180           | 45         | 6                | 11.0 |
|    | 0.5      |                   | 20            | 20         | 3                |      |

<sup>1</sup> Times kappa.

Corresponding cooks and bleaches were carried out subsequent to storing the chips according to the invention. It was shown that the chips treated with micro-organisms according to the invention presented a total loss in weight of 1.3% whereas the untreated chips showed a loss in weight of 2.2%. The weight loss of the untreated portions must be considered low since the "normal" value for losses in weight can lie between 3-4%. The reasons why the values were so low in this case was due to the fact that all the surrounding chips had been treated and thus protected the untreated chip portions from deleterious micro-organisms.

On analysis of micro-flora present in the pile of wood chips it was seen that in the outer portions of the pile, where the low-temperature fungus *Gliocladium viride* had been active, the protective effect by anti-biosis had been complete. The amount of rot fungi in the inner portion of the pile was very slight. The total protective

effect had thus been very good. The extract content (DKM) of chips treated according to the invention, and unbleached and bleached sulphite pulp produced from said chips, was 0.70, 0.85 and 0.13%. Corresponding values for untreated chips and unbleached and bleached sulphite pulp produced from said chips was 0.90, 1.30 and 0.20%.

Concerning other analysis values no difference could be noted with pulp produced from chips treated according to the invention or with pulps produced from chips stored in the conventional manner.

We claim:

1. A process for storing wood chips under conditions such that resinous components present in the chips are subjected to enzymatic hydrolysis induced by fungi added to the chips while minimizing microbial action on cellulose and hemicellulose in the wood, which comprises adding to the wood chips a fungus or fungi capable of elaborating esterases which attack ester linkages in the wood resinous components and which either completely or partly lack the ability of elaborating active cellulases, selected from the group consisting of:

(1) fungi which inhibit cellulose- and hemicellulose-decomposing microorganisms by developing a high temperature in the wood chips inhibiting propagation of such micro-organisms, selected from

*Humicola grisea* var. *thermoidea*, characterized by Cooney-Emerson

*Humicola stellata*, characterized by Bunce

*Humicola insolens*, characterized by Cooney-Emerson

*Humicola languinosa*, characterized by Griffon-Maublanc-Bunce

*Talaromyces duponti*, characterized by Griffon-Maublanc-Cooney-Emerson

*Thermoascus aurantiacus*, characterized by Miehe

*Mucor pusillus*, characterized by Lindt

*Mucor miehei*, characterized by Cooney-Emerson

*Malbranchea pulchella*, Saccardo-Penzig var. *sulfurea*, characterized by Miehe

*Myriococcum albomyces*, characterized by Cooney-Emerson

*Sporothrix thermophile*, characterized by Apinis

*Allescheria terrestris*, characterized by Apinis

5

10

15

20

25

30

35

40

45

*Torula thermophile*, characterized by Cooney-Emerson

*Chaetomium thermophile*, characterized by La Touche

*Stilbella thermophile*, characterized by Fergus

*Aspergillus fumigatus*, characterized by Fresenius

(2) fungi which inhibit cellulose- and hemicellulose-decomposing micro-organisms by antibiotic effect, selected from:

*Trichoderma Lingnorum*, characterized by Tode-Harz

*Gliocladium roseum*, characterized by Link-Thom

*Gliocladium deliquescent*, characterized by Sopp

*Penicillium funicolosum*, characterized by Thom

*Penicillium roqueforti*, characterized by Thom

*Penicillium rubrum*, characterized by Stoll

*Gliocladium viride*, characterized by Stoll

and

(3) fungi selected from:

*Dactyloomyces thermophilus*

*Rhizopus arrhizus*

and then storing the wood chips in a pile under conditions favorable to the growth of the added fungus or fungi.

2. A process in accordance with claim 1 in which the fungi are added to the wood chips in the form of an aqueous dispersion of the spores thereof.

3. A process in accordance with claim 1 in which the fungus is especially selected to propagate at low winter temperatures.

4. A process in accordance with claim 1 in which the fungi are applied to the chips in the form of an aqueous dispersion which is sprayed over the chips.

#### References Cited

#### UNITED STATES PATENTS

|           |        |          |       |         |
|-----------|--------|----------|-------|---------|
| 1,633,594 | 6/1927 | Lathrop  | ----- | 195—8 X |
| 2,193,493 | 3/1940 | Ritter   | ----- | 195—10  |
| 2,871,163 | 1/1959 | Turnbull | ----- | 195—8   |
| 3,401,085 | 9/1968 | Croon    | ----- | 162—1 X |

HOWARD R. CAINE, Primary Examiner

U.S. Cl. X.R.